

(Model.)

C. GRAHAM.

DECORATION OF POTTERY WARE.

No. 315,021.

Patented Apr. 7, 1885.

Fig. 6

Fig. 2.



Fig. 1.



Fig. 5.



Fig. 3.



Fig. 4.



WITNESSES—

Charles R. Searle,  
M. F. Boyle

INVENTOR—

Charles Graham  
by his attorney  
Thomas D. Peterson.

# UNITED STATES PATENT OFFICE.

CHARLES GRAHAM, OF BROOKLYN, NEW YORK.

## DECORATION OF POTTERY-WARE.

SPECIFICATION forming part of Letters Patent No. 315,021, dated April 7, 1885.

Application filed August 28, 1884. (Model.)

*To all whom it may concern:*

Be it known that I, CHARLES GRAHAM, of Brooklyn, Kings county, in the State of New York, have invented certain new and useful 5 Improvements in the Decoration of Pottery-Ware, of which the following is a specification.

I have discovered that by proper manipulation glazing may be removed entirely at certain points by a process analogous to the etching of metals, and without much eating into or affecting the burned clay lying under it. I have successfully applied this in the development of an important improvement in the arts.

I take white or light cream or other light-colored ware and glaze it uniformly with salt-glaze, under conditions which will give a black, chocolate, or other dark shade. I then cover the surface with a ground of wax or analogous matter, which may be the same as is commonly used in etching on copper or steel. I then transfer to the surface from a previously-made drawing or print the outline of the figures to be etched, and remove the ground on the desired points or along the lines which it is desired to bite, and immerse the whole in dilute hydrofluoric acid, using the acid of a strength one part acid and two parts water. After an exposure to this acid for about ten minutes the article is taken out, washed with water 25 containing ammonia, and the ground being removed with turpentine or by other suitable means the points and lines will appear in white or the light color of the biscuit, while the remaining portions of the surface glazing 30 will remain unaffected.

Instead of applying the ground over the whole surface at the beginning, I can, and in working in the large way I propose in many or most cases, to operate as follows: Prepare a 40 plate, which may be a plane plate of copper, glass, or other suitable material having the lines cut or etched deeply therein, and apply to this plate the ground, preferably for this purpose using asphalt, or a composition of 45 which the asphalt of Trinidad or analogous material is a principal constituent. Then removing, by scraping or otherwise, all the ground except what remains in the lines, I apply dampened paper, and impress by passing it 50 through between the rollers of a plate-printing press. On removing the paper the ground

will lie thereon in the proper lines. Now, on applying this to the previously-glazed ware, and pressing gently over the exterior by what is known as "rubbing," and removing the 55 paper, the ground will lie on the ware in the required lines. The effect produced by biting will be the same as that on the paper. The lines will be dark on white ground.

If it is desired to make the lines white on 60 dark ground, a similar process can be used, making all the lines in the pattern-plated double, so as to inclose between them an unaffected line, which will represent the line to be finally produced in white on the darkly-glazed ware. 65 The filling with a coating of the asphalt between the bordering of the lines thus produced will be applied by hand after the paper has been removed from the ware.

I will represent the invention as carried out 70 in the manner last described.

The accompanying drawings form a part of this specification.

Figure 1 is a side view of a stoneware bottle decorated according to my invention. The 75 remaining figures are on a larger scale. Fig. 2 shows a portion covered with the ground, with the desired lines traced or otherwise cut through the ground. Fig. 3 shows the same immersed in acid with the chemical reaction 80 going on. Fig. 4 shows the resulting condition after the operation is completed and the etching-ground has been removed. Figs. 5 and 6 represent an intermediate stage of the work. Fig. 5 is a section through the paper 85 after it has received the outlines in asphalt from an engraved plate. (Not represented.) Fig. 6 shows the ware after the asphalt has been transferred thereto from the paper, but before the spaces between the outlines have been 90 filled in by hand.

The thickness of the coating of asphalt or other ground, as also the thickness of the glaze and the depth to which the acid bites, are all 95 exaggerated in the figures to show the peculiarities more distinctly.

Similar letters of reference indicate corresponding parts in all the figures where they occur.

A is the cream-colored body of the crockery; 100 B, a dark salt-glaze; C, the ground of wax, bitumen, or analogous material adapted to re-

sist the action of the acid; D, the acid, and d the bubbles of gas due to the combination of the acid with the material of the glazing. E is the paper.

5 I believe that I can afterward immerse the ware in any ordinary glazing to reglaze the whole surface, including the portions thus exposed. Care being taken to avoid the running of the two glazings into each other, the 10 effect will be very fine. I have not in my experiments deemed it necessary to reglaze the ware. I have left the dark glazing as a ground, the light lines clearly depicted on it being sunk to the extent of the thickness of 15 the glazing and a little more, and the surface of the body thus exposed being left unglazed.

Modifications may be made. I can treat articles of other shapes and designated by other names than the bottle shown. I can employ 20 a body of dark gray or dark red with a glazing of lighter hue. I can vary the character of the glazing within considerable limits. It is only essential that there shall be a marked contrast between the body A and the glaze B, 25 and that the glaze shall be of a character which is attacked and removed by the acid while the body will not be much affected thereby. A slight biting of the acid into the body will not be a serious evil. I have determined by 30 experiment that the operation, if managed with reasonable care, will not materially under-cut the glaze so as to injure the pottery.

Instead of one part anhydrous acid to two parts water, I can succeed well with some 35 ware using considerably more diluted acid—say one part acid to three parts water. The strength of the acid and the time of exposure will vary with different glazes. The operation will be completed sometimes in less than 40 five minutes. Other glazes will require a longer period, even up to an hour.

It may not be necessary in all cases to use damp paper, or to use a printing-press, to sufficiently receive the impression of "ground" from the printing-surface and transfer it. 45

In some cases I design to further ornament the pottery by peculiarly treating the etched surfaces; but such process will be made subject-matter for separate application.

I claim as my invention—

1. The method described of decorating ceramic ware by coating with a glaze presenting a different color or shade from the body, and etching through the said glaze at points or lines so as to expose the ground in contrast therewith, thereby presenting ornamental or distinguishing figures, substantially as herein specified. 55

2. The method described of decorating cylindrical and analogous surfaces of pottery by printing the desired figures, with ground adapted to resist the action of acid, transferring the same by paper or analogous flexible material to the surfaces previously glazed, filling by hand between the lines if necessary, 65 and then exposing to acid until the glazing is bitten through at the exposed points, substantially as herein specified.

3. Ceramic ware having a body and glazing of different tints or shades with the glazing removed in ornamental or distinguishing figures, so as to present a body in contrast therewith, as herein specified. 70

In testimony whereof I have hereunto set my hand, at New York city, New York, this 75 23d day of August, 1884, in the presence of two subscribing witnesses.

CHAS. GRAHAM.

Witnesses:

J. E. RENWEE,  
CHARLES R. SEARLE.